

## UNITED STATES PATENT OFFICE.

EDWIN F. KINGSBURY, OF RUTHERFORD, NEW JERSEY, ASSIGNOR TO WESTERN ELECTRIC COMPANY, INCORPORATED, OF NEW YORK, N. Y., A CORPORATION OF NEW YORK.

## METALLIC COMPOSITION.

No Drawing.

Application filed August 14, 1923. Serial No. 657,435.

*To all whom it may concern:*

Be it known that I, EDWIN F. KINGSBURY, a citizen of the United States of America, residing at Rutherford, in the county of Bergen, State of New Jersey, have invented certain new and useful Improvements in Metallic Compositions, of which the following is a full, clear, concise, and exact description.

10 This invention relates to metallic compositions, and particularly to contact alloys; and its object is to provide a satisfactory metal for use as a wire contact member.

In accordance with the features of the invention, there is provided a metallic composition which will give efficient service when formed into grid wires for co-ordinate switches such as employed in automatic telephone impulse-sending apparatus.

20 It is necessary that such a metal have a low contact resistance, a maximum life in spite of the mechanical wear to which it is subjected, and but little tendency to be electrically corroded by arcing especially when used with the usual phosphor-bronze contact members of co-ordinate switches. The metal should also be tough, reasonably cheap, and comparatively homogeneous, and should have a good tensile strength. It 30 should also be of such a character that it will not cause contact members composed of such a metal as phosphor-bronze to be rapidly worn out.

It has been found that a metallic composition comprising about 10 to 50 per cent

of silver, about 1½ to 5 per cent of tin, and about 45 to 88 per cent of copper possesses these qualities to a marked degree and is exceedingly satisfactory for use as grid wire to be employed with phosphor-bronze contacts in co-ordinate switches or similar apparatus. An alloy containing these metals in the following proportions has proved the most satisfactory for this purpose, silver 15 per cent, tin 2 per cent, 40 and copper 83 per cent. The tin content, however, may be raised to 4 per cent and the copper content correspondingly decreased without any marked change in the efficiency of the alloy. 45

The invention claimed is:

1. A metallic composition comprising as the essential elements thereof the following metals in substantially the following proportions, silver 10 to 50 per cent, tin 1½ to 5 per cent, and copper 45 to 88 per cent. 55

2. A contact alloy comprising as the essential elements thereof the following metals in substantially the following proportions, silver 15 per cent, tin 2 to 4 per cent, and copper 81 to 83 per cent. 60

3. A grid wire to be used with phosphor-bronze contact members, which is composed of the following metals in substantially the following proportions, silver 15 per cent, tin 2 per cent, and copper 83 per cent. 65

In witness whereof I hereunto subscribe my name this 8th day of August, A. D., 1923.

EDWIN F. KINGSBURY.